

## 1

3,276,877

 METHOD OF PREPARING SENSITIZED  
PHOTOGRAPHIC EMULSIONS

Henry Clay Yutzy and William F. Smith, Rochester, N.Y., assignors to Eastman Kodak Company, Rochester, N.Y., a corporation of New Jersey  
No Drawing. Filed July 17, 1964, Ser. No. 383,508  
4 Claims. (Cl. 96—108)

This application is a continuation-in-part of our applications Serial Nos. 526,321, filed August 3, 1955 and 235,555, filed November 5, 1962, both now abandoned.

This invention relates to photographic emulsions having a particle crystal dislocation value of less than 5 per micron<sup>2</sup> of surface area which emulsions upon exposure form a surface image but little or no internal image, a process for preparing those emulsions and the reversal development of those emulsions.

It is known that the silver halide crystals of the usual photographic emulsions are considerably sensitive to light both internally and on the surface. Photographic emulsions up to the time of this invention have been those having a concentration of dislocations per micron<sup>2</sup> of silver halide surface area considerably more than 5.0 and generally greater than 10 dislocations per micron<sup>2</sup>. In certain types of photographic processes it has appeared desirable to employ emulsions in which the surfaces of the silver halide crystals have a sensitivity considerably greater than the internal portions thereof.

One object of our invention is to provide photosensitive silver halide emulsions characterized in that the concentration of dislocations is less than 5.0 per micron<sup>2</sup> of surface area, which emulsions are characterized by low internal sensitivity of the silver halide crystals thereof. Another object of our invention is to provide a process for preparing photosensitive silver halide emulsions having a low concentration of dislocations. A further object of our invention is to provide a method for preparing emulsions which are eminently suited for use in reversal photography both color and black-and-white types. A still further object of our invention is to provide a process involving the reversal development of photographic emulsions having a low particle crystal dislocation value. Other objects of our invention will appear herein.

In accordance with our invention an emulsion is obtained the surface sensitivity of the silver halide crystals of which when developed in a surface developer and measured at a density of 0.1 plus fog is greater by at least 1.75 log E than the internal sensitivity of those crystals as measured by the development thereof, after bleaching, in an internal developer. These emulsions are characterized by having less than 5.0 dislocations per micron<sup>2</sup> of surface area. The determination of particle crystal dislocation values is described in an article entitled "Convergent-Beam X-Ray Analysis of Mosaic Structure in Polycrystals" by Chester R. Berry which appeared in the Journal of Applied Physics, Volume 27, No. 6, pages 636-639, June 1956. The emulsions in accordance with our invention are characterized by a physical structure in which the concentration of dislocations is less than 5.0 per micron<sup>2</sup> of surface area which value is readily determined by the simple diffraction method as described in that article. As recognized in that article, many schemes have been proposed for determining angular misalignment in crystals and the invention is not limited to the determination described in the Berry article.

The physical structure of the silver halide crystals of sensitized photographic emulsions governs the relation of their surface sensitivity to their internal sensitivity, the surface sensitivity of those crystals having a dislocation value of less than 5.0 dislocations per micron<sup>2</sup> of

## 2

surface area being greater by at least 1.75 log E than the internal sensitivity thereof as measured by comparing the result obtained by developing after exposure in a surface developer with developing in an internal developer, the latter after first bleaching in 0.3% potassium ferricyanide solution and drying. A typical surface development involves developing the emulsion after exposure for 6 minutes at 68° F. in a developer having the following formula:

|    |                               |       |      |
|----|-------------------------------|-------|------|
| 10 | Water                         | cc    | 750  |
|    | Elon                          | grams | 0.31 |
|    | Sodium sulfite (desiccated)   | do    | 39.6 |
|    | Hydroquinone                  | do    | 6.0  |
| 15 | Sodium carbonate (desiccated) | do    | 18.7 |
|    | Potassium bromide             | do    | 0.86 |
|    | Citric acid                   | do    | 0.68 |
|    | Potassium metabisulfite       | do    | 1.5  |
|    | Cold water to make 1.0 liter. |       |      |

20 A typical internal development involves first bleaching the emulsion layer after exposure in aqueous 0.3% potassium ferricyanide solution and drying and then developing for 5 minutes at 65° F. in an internal developer having the following composition:

|    |                               |       |     |
|----|-------------------------------|-------|-----|
| 25 | Water                         | cc    | 500 |
|    | Elon                          | grams | 2.2 |
|    | Desiccated sodium sulfite     | do    | 96  |
|    | Hydroquinone                  | do    | 8.8 |
| 30 | Desiccated sodium carbonate   | do    | 48  |
|    | Potassium bromide             | do    | 5   |
|    | Sodium thiosulfate            | do    | 10  |
|    | Cold water to make 1.0 liter. |       |     |

25 Defined in photographic terms the emulsions in accordance with our invention have a surface sensitivity greater by at least 1.75 log E measured at a density of 0.1 plus fog than the internal sensitivity. In physical terms the emulsions in accordance with our invention have less than 5.0 dislocations per micron<sup>2</sup> of surface area as determined by a method for determining the substructure or angular misalignment in crystals such as by the simple X-ray diffraction method described by Berry in his article referred to above.

30 We have found that silver halide crystals of emulsions in accordance with our invention are obtained by processes in which the following conditions are observed:

35 (1) Ammoniacal silver nitrate and alkali halide are passed simultaneously into a solution of gelatin or a gelatin derivative with stirring.

40 (2) At least 50% of the alkali halide is added to the solution of gelatin or gelatin derivative while the solution of ammoniacal silver nitrate is being introduced. The best results are obtained when the alkali metal halide is present in but small excess in the solution of gelatin or gelatin derivative. For instance, an excess of no more than about 5 mole percent of the silver present in the reaction mixture.

45 (3) The emulsion is of the bromoiodide type, the iodide being preferably 0.5-5 mole percent based on the total silver halide in the emulsion.

50 (4) The emulsion is chemically sensitized to increase its surface sensitivity. In some cases the chemical sensitizer, e.g. sulfur sensitizer, may be contained in the protein material used in preparing the emulsion.

55 The best results are obtained with the simultaneous addition of the alkali metal halide and the silver nitrate to the gelatin or gelatin derivative solution within a period of no more than 20 minutes.

60 The ammoniacal silver nitrate used is prepared by adding to an aqueous solution of silver nitrate an amount of ammonia sufficient to precipitate the silver as silver oxide and to redissolve the same preferably with a slight

excess of ammonia. The alkali halide solution is usually prepared by dissolving in water both the alkali metal bromide and alkali metal iodide. The solution to which the alkali halide and the silver nitrate are added is a solution in water of protein or protein derivative, usually gelatin or its derivative at a concentration of 0.5-5%. The silver halide dispersion may be washed by one of the processes known in the art such as chill setting and washing by osmosis or by one of the coagulation techniques, such as described in U.S. Patents 2,618,556, 2,614,928 and 2,489,-341. In the preparation of the silver halide the protein material can be gelatin or it can be oxidized casein such as described in U.S. Patent 2,691,582 of Lowe and Gates.

It is preferable to add the silver nitrate solution and alkali halide solution simultaneously to the aqueous solution of protein or its derivative over substantially the entire time of addition. If desired separate solutions of alkali metal bromide and alkali metal iodide may be employed provided they are added substantially simultaneously to the protein solution, the operation being carried out so that most of the time the alkali metal halide is present in the protein solution in small excess.

After the silver halide has been prepared and washed as mentioned above, it is then dispersed in a vehicle which is usually gelatin and is chemically sensitized. The chemical sensitization of silver halide emulsions is well known in the art and refers to increasing the surface sensitivity of the emulsion by reacting the silver halide with sulfur, selenium, or tellurium compounds as described in U.S. Patents 1,574,944, 1,623,499, and 2,410,689 of Sheppard, or by reacting the silver halide with noble metals such as gold, palladium or platinum as described in U.S. Patent 2,448,060 and British Patent No. 636,140 of Trivelli and Smith, or by reacting the silver halide with reducing agents as described in Carroll British Patent 658,592 and Lowe and Jones U.S. Patent 2,518,698, or by various combinations of these as described in Waller et al. U.S. Patent 2,399,083 and Lowe et al. U.S. Patents 2,743,182 and 2,743,183. Optionally the emulsions may be sensitized with polyethylene glycols such as described in U.S. Patents 2,423,459; 2,441,389; 1,970,578; 2,400,532, 2,240,472 or British Patent 443,559. The emulsion may be ripened at an elevated temperature for a time sufficient to impart the desired properties to the emulsion. After the emulsion has been prepared, it may be coated out onto a support such as a film base of cellulose triacetate, cellulose acetate propionate or the like.

The low crystal dislocation emulsions which are characterized by high surface, low internal sensitivity are primarily employed in photographic films designed for reversal development such as for color films as referred to in U.S. Patents 2,172,262 and 2,252,718 or for mixed grain color films of the type described in U.S. Patents 2,592,243 and 2,673,149. Mixed grain emulsions of this type may be developed as described in U.S. Patent 2,614,925.

Emulsions in accordance with our invention may also be employed in the manufacture of films sensitized to various regions of the spectrum which are adapted for reversal development and in the manufacture of black and white films adapted for use in reversal development processes of the type described in U.S. Patent 1,460,703 of Capstaff.

#### EXAMPLE I

This example describes a method of preparing emulsions having an appreciable number of dislocations per particle which emulsion is characterized by a low ratio of surface to internal sensitivity for comparison with emulsions in accordance with our invention. The concentration of dislocations per micron<sup>2</sup>

$$\frac{(\Delta 2\theta)}{bD \times 10^8}$$

was determined in accordance with the method described in Berry's article. The concentration of dislocations per

micron<sup>2</sup> was found to be 14. In this definition D is the average diameter of the silver halide crystals in microns, b is the length of the Burger's vector and  $\Delta 2\theta$  is the width of a spot produced near the wide part of the diffraction ring as described in Berry's article.

#### Solution A

52 grams of a photographic gelatin, 250 grams of potassium bromide, 3.5 grams of potassium iodide; dissolved in 4500 cc. of distilled water at 50° C.

#### Solution C

340 grams of silver nitrate were dissolved in distilled water making a total volume of 2750 cc. The temperature was adjusted to 40° C.

15 Solution C was run into Solution A in approximately 45 minutes with good stirring. The mixture was cooled to 30° C. and the emulsion was acidified by the addition of 6 N sulfuric acid. The emulsion was rendered substantially free of residual water soluble salts by washing by a conventional coagulation technique. After washing, 428 grams photographic gelatin and sufficient distilled water were added to make a total weight of 6.5 kilograms. The mixture was stirred at 40° C. at a pH of 6.4 until 20 completely dispersed. The emulsion was then chemically sensitized as described in Example 5 of British Patent 636,234, except the sulfur and gold compounds were added before the second digestion. After digesting to 25 optimum sensitivity, the following coatings were made.

30 (A) A portion of the emulsion was coated on a cellulose acetate support at a coverage of 570 sq. ft. per mole of silver halide. Separate samples of this coating were exposed on an Eastman 1B Sensitometer; one was processed in the surface developer and the other was 35 bleached with alkali metal ferricyanide and was processed in the internal developer, previously described. The log of the exposure measured at a density of 0.1+fog of the coating processed in the internal developer, was found to be log E=less than 1.75 slower than the strip 40 processed in the surface developer.

(B) Two separate portions of this emulsion were divided out. A red sensitizer was added to one portion and a green sensitizer was added to the second portion. These two portions were blended together and coated as a single layer on a cellulose acetate support as described in the 45 Carroll and Hanson U.S. Patents 2,592,243 and 2,673,149 resulting in a mixed grain color film.

#### EXAMPLE II

This example illustrates the preparation of an emulsion 50 in accordance with our invention which emulsion is characterized by a high ratio of surface to internal sensitivity and the concentration of dislocations per micron<sup>2</sup> of surface area was determined to be 4.8 by the simple X-ray diffraction method described in Berry's article. The average grain size of the silver halide grains obtained was less than 1 micron diameter.

#### Solution A

52 grams of a photographic gelatin were dissolved in 60 3500 cc. of distilled water at 40° C.

#### Solution B

250 grams of potassium bromide, and 3.5 grams of potassium iodide were dissolved in sufficient distilled water to make a total volume of 1020 cc. at 40° C.

#### Solution C

340 grams of silver nitrate were dissolved in 1600 65 grams of distilled water; 300 cc. of 28% ammonium hydroxide were added and the total volume was adjusted to 2850 cc. with distilled water and the temperature was raised to 40° C.

Solutions B and C were run into Solution A in approximately 11 minutes with good stirring. The running of Solution B was started 15 seconds before that of Solution

C. After the addition of B and C the mixture was cooled to 30° C. and the emulsion was acidified by the addition of 6 N sulfuric acid. The emulsion was rendered substantially free of residual water soluble salts by washing by a conventional coagulation technique and after washing, 428 grams of photographic gelatin and sufficient distilled water were added, to make a total weight of 6.5 kilograms. The mixture was stirred at 40° C. and at a pH of 6.4 until completely dispersed. The emulsion was chemically sensitized as in the previous example. The emulsion was digested to optimum sensitivity and the following coatings were made:

(A) A portion of the above emulsion was coated on a cellulose acetate support at a coverage of approximately 570 sq. ft. per mole of silver halide. Samples of this coating were exposed and processed in internal and surface developers as described in Example I and this emulsion was found to have a surface sensitivity  $\log E = 2.0$  greater than the internal sensitivity when measured at a density of 0.1+fog in the manner previously described.

(B) Separate portions of this emulsion were red and green sensitized respectively and a mixed grain color coating was made as described in Example I in part B.

### EXAMPLE III

The pressure sensitivity of the coatings described above were determined by placing a strip of each coating on a rigid metal surface and running a narrow weighted wheel along the center of the coating. The diameter of the wheel was  $1\frac{1}{16}$  in. and the width of the wheel was  $\frac{1}{32}$  in. A weighted arm attached to a fulcrum rested on the wheel. The weight at the end of the arm was 2035 grams, and the distance along the arm from the wheel to the fulcrum was 1 inch. The distance from the fulcrum to the weight was  $23\frac{1}{2}$  in. After the coatings were pressured by the wheel in the manner described, the strips were exposed on a sensitometer. The exposure was such that part of the sensitometric strip was in the pressured region and part of the strip was in the untreated region, so that the sensitometric characteristics of both regions could be determined. This was done with the following results:

(a) The single layer film coatings described in Examples I-A and II-A were exposed and developed to a cyan reversal image as follows:

- (1) Preconditioning 24 hrs. at 50% R.H.
- (2) Pressure wheel run down center of strip.
- (3) Sensitometric exposure.
- (4) MQ developer, 3 min.
- (5) Wash, 2 min.
- (6) White light re-exposure. 10 seconds through base.
- (7) Cyan color developer, 5 min.
- (8) Wash—5 min.
- (9) Bleach—3 min.
- (10) Fix—2 min.
- (11) Wash—10 min.

The pressure characteristics of these coatings are tabulated below. The changes in maximum density, the change in high-light density and the  $\log E$  changes measured at a 0.2 density above fog of the untreated film are as follows:

| Coating     | Change in Maximum Density | Change in High-Light Density | Change in $\log E$ measured at 0.2 Above Fog |
|-------------|---------------------------|------------------------------|----------------------------------------------|
| Example IA  | -.08                      | +.12                         | -.45                                         |
| Example IIA | -.08                      | 0                            | 0                                            |

(b) These two coatings were also processed in the following black and white reversal system with the indicated results:

- 6
- (1) Precondition 24 hrs. at 50% R.H.
  - (2) Pressure wheel run down center of strip.
  - (3) Sensitometric exposure.
  - (4) MQ developer—3 min.
  - (5) Wash—2 min.
  - (6)  $KM_nO_4$  bleach—4 min.
  - (7) Clearing bath—3 min.
  - (8) Wash—3 min.
  - (9) White light re-exposure—10 seconds.
  - (10) Redeveloper—5 min.
  - (11) Acid fix—3 min.
  - (12) Wash—10 min.

| Coating     | Change in Maximum Density | Change in High-Light Density | Change in $\log E$ measured at 0.2 Above Fog |
|-------------|---------------------------|------------------------------|----------------------------------------------|
| Example IA  | -.02                      | +.04                         | -.16                                         |
| Example IIA | -.09                      | -.02                         | +.02                                         |

(c) The mixed grain coatings described above were processed in the following mixed grain reversal process with the indicated results:

- (1) Preconditioning 24 hrs. at 50% R.H.
- (2) Pressure wheel run down center of strip
- (3) Sensitometric exposure
- (4) MQ developer—3 min.
- (5) Wash—2 min.
- (6) Red re-exposure through red filter—5 seconds
- (7) Cyan color developer—5 min. 50 seconds
- (8) Auxiliary developer—50 seconds
- (9) Wash—1 min.
- (10) Green re-exposure through yellow filter—30 seconds
- (11) Magenta color developer—5 min.
- (12) Wash—5 min.
- (13) Bleach—3 min.
- (14) Fix—2 min.
- (15) Wash—10 min.

| Coating               | Change in Maximum Density | Change in High-Light Density | Change in $\log E$ measured at 0.2 Above Fog |
|-----------------------|---------------------------|------------------------------|----------------------------------------------|
| Example IB (Cyan)     | -.18                      | +.06                         | -.20                                         |
| Example IIB (Cyan)    | -.03                      | 0                            | +.02                                         |
| Example IB (Magenta)  | -.14                      | +.06                         | -.12                                         |
| Example IIB (Magenta) | -.03                      | 0                            | +.03                                         |

50 It can be seen quite clearly from the above results that emulsions having a high ratio of surface to internal sensitivity are much less sensitive to pressure than emulsions having a low ratio of surface to internal sensitivity. The solutions used for processing the coatings in Example III are as follows:

#### MQ developer:

|                           |    |      |
|---------------------------|----|------|
| Sodium hexa metaphosphate | gm | .5   |
| $Na_2SO_3$                | gm | 40.0 |
| Elon                      | gm | 5.0  |
| HQ                        | gm | 2.0  |
| $Na_2CO_3$                | gm | 25.0 |
| NaBr                      | gm | .86  |
| $Na_2SO_4$                | gm | 25.0 |
| KI                        | gm | .002 |
| pH                        |    | 10.0 |
| Sp-Gr.                    |    | 1.08 |

#### Cyan color developer:

|                                               |            |      |
|-----------------------------------------------|------------|------|
| $H_2SO_4$ conc.                               | cc. (app.) | .9   |
| Sodium hexa metaphosphate                     | gm         | .5   |
| $Na_2SO_3$                                    | gm         | 5.0  |
| 2-amino-5-diethyl amino toluene hydrochloride | gm         | .55  |
| $Na_2CO_3$                                    | gm         | 15.0 |
| NaBr                                          | gm         | .22  |

|                                                                                                  |       |       |
|--------------------------------------------------------------------------------------------------|-------|-------|
| 6-nitrobenzamidazol nitrate                                                                      | gm    | .02   |
| KI                                                                                               | gm    | 0.002 |
| Hydroxylamine hydrochloride                                                                      | gm    | 1.5   |
| 2,4-dichloro-5-(p - toluene sulfonyl amino-1-naphthol)                                           | gm    | .5    |
| NaOH                                                                                             | gm    | .5    |
| pH                                                                                               | ----- | 10.0  |
| Auxiliary developer:                                                                             |       |       |
| Sodium hexa metaphosphate                                                                        | gm    | 1.0   |
| Na <sub>2</sub> SO <sub>3</sub>                                                                  | gm    | 20.0  |
| Elon                                                                                             | gm    | 3.0   |
| Na <sub>2</sub> CO <sub>3</sub>                                                                  | gm    | 25.0  |
| NaBr                                                                                             | gm    | 4.3   |
| NaOH                                                                                             | gm    | 1.55  |
| 6-nitrobenzamidazol nitrate                                                                      | gm    | .1    |
| pH                                                                                               | ----- | 11.5  |
| Magenta color developer:                                                                         |       |       |
| Sodium hexa metaphosphate                                                                        | gm    | .5    |
| Na <sub>2</sub> SO <sub>3</sub>                                                                  | gm    | 5.0   |
| 4-amino, N-ethyl, N-(beta-methane sulfonamido - ethyl) - m - toluidine sesquisulfate monohydrate | gm    | 3.5   |
| Na <sub>2</sub> CO <sub>3</sub>                                                                  | gm    | 20.0  |
| KBr                                                                                              | gm    | .22   |
| Na <sub>2</sub> SO <sub>4</sub>                                                                  | gm    | 50.0  |
| 6-nitrobenzamidazol nitrate                                                                      | gm    | .01   |
| KI                                                                                               | gm    | .002  |
| 1-(2' - quinolyl) - 3 - benzamido - 5 - pyrazolone                                               | gm    | 1.0   |
| NaOH                                                                                             | gm    | .8    |
| pH                                                                                               | ----- | 10.7  |
| Bleach:                                                                                          |       |       |
| Sodium hexa metaphosphate                                                                        | gm    | 1.0   |
| K <sub>3</sub> FE(CN) <sub>6</sub>                                                               | gm    | 80.0  |
| NaBr                                                                                             | gm    | 34.4  |
| Fix:                                                                                             |       |       |
| Sodium hexa metaphosphate                                                                        | gm    | 10.0  |
| Na <sub>2</sub> SO <sub>3</sub>                                                                  | gm    | 10.0  |
| Sodium thiosulfate                                                                               | gm    | 320.0 |
| KMnO <sub>4</sub> bleach:                                                                        |       |       |
| KMnO <sub>4</sub>                                                                                | gm    | 2.5   |
| H <sub>2</sub> SO <sub>4</sub>                                                                   | cc    | 15.5  |
| AgNO <sub>3</sub>                                                                                | gm    | 0.3   |
| Clearing bath:                                                                                   |       |       |
| Sodium hexa metaphosphate                                                                        | gm    | 0.6   |
| NaHSO <sub>3</sub>                                                                               | gm    | 15.0  |
| Redeveloper:                                                                                     |       |       |
| Sodium hexa metaphosphate                                                                        | gm    | 0.6   |
| Na <sub>2</sub> SO <sub>3</sub>                                                                  | gm    | 70.0  |
| Elon                                                                                             | gm    | 1.45  |
| Hydroquinone                                                                                     | gm    | 5.6   |
| Na <sub>2</sub> CO <sub>3</sub>                                                                  | gm    | 39.7  |
| KBr                                                                                              | gm    | 1.1   |
| Acid fix:                                                                                        |       |       |
| Sodium thiosulfate                                                                               | gm    | 240.0 |
| Sodium sulfite, desiccated                                                                       | gm    | 15.0  |
| Acetic acid, 28%                                                                                 | cc    | 48.0  |
| Boric acid, crystals                                                                             | gm    | 7.5   |
| Potassium alum                                                                                   | gm    | 15.0  |

## EXAMPLE IV

This example is another example of a method of preparing photographic emulsions having less than 5.0 dislocations per micron<sup>2</sup> of surface area. The concentration of dislocations per micron<sup>2</sup> of surface area was determined by the X-ray diffraction method described in Berry's article and was found to be 4.8.

## Solution A

525 grams of a photographic gelatin were dissolved in 8750 cc. of distilled water at 45° C.

## Solution B

625 grams of potassium bromide and 8.75 grams of potassium iodide were dissolved in distilled water to form a total volume of 2440 cc. at 40° C.

## Solution C

850 grams of silver nitrate were dissolved in 4000 cc. of distilled water. There was then added 750 cc. of 28% ammonium hydroxide by which a precipitate was formed and was redissolved. The volume of the solution was brought to 6750 cc. by adding distilled water at a temperature of 40° C.

Solutions B and C were run simultaneously into Solution A over a period of approximately 11 minutes, the addition of Solution B having been started 15 seconds before that of Solution C. The mass was stirred mechanically during the mixing. After the formation of the silver halide dispersion the mass was cooled to 28° C. and the emulsion was acidified by the addition of 6 N sulfuric acid. The emulsion was rendered substantially free of residual water soluble salts by washing by a conventional coagulation technique. After washing 875 grams of photographic gelatin and sufficient distilled water were added to make a total weight of 19.5 kilograms. The emulsion was dispersed at 40° C. and at a pH of 6.4 and 285 cc. of a 10% solution salicylamide in methyl alcohol were added. The emulsion was chemically sensitized as described in Example 5 of British Patent 636,234 except the compounds were added before the second digestion. Saponin was added as a coating aid and the emulsion mass was applied as a layer onto a subbed cellulose acetate film support at the rate of 570 sq. ft. per mol of silver halide.

## EXAMPLE V

This example is offered as a method of preparing photographic emulsions in accordance with our invention. The concentration of dislocations per micron<sup>2</sup> of surface area of the emulsion grains thus prepared was found to be 4.0 when the emulsion thus prepared was examined by the X-ray diffraction method described in Berry's article. These grains had an average size of less than 1 micron diameter.

## Solution A

52 grams of a photographic gelatin were dissolved in 3500 cc. of distilled water at 45° C.

## Solution B

25 grams of potassium bromide and 3.5 grams of potassium iodide were dissolved in 90 cc. of distilled water at 40° C.

## Solution C

340 grams of silver nitrate were dissolved in 1600 cc. of distilled water and there was added thereto 300 cc. of 28% ammonium hydroxide which addition caused the formation of a precipitate and redissolving thereof. The total volume was adjusted to 2700 cc. by adding distilled water at 40° C.

## Solution E

225 grams of potassium bromide were dissolved in 790 cc. of distilled water at 40° C.

Solutions B and C were run into Solution A with good mechanical stirring, the introduction of Solution B having been started approximately 10 seconds before Solution C. Solution B was run in completely over 1 minute and then Solution E was run into Solution A, this taking approximately 9 minutes. The running of Solution C into A was over a period of 11 minutes so that the halides and the silver solution were both run into Solution A over substantially the entire period. After the solutions had all been mixed together the mass thus formed was allowed to cool to 28° C. and was then acidified by the addition of 6 N sulfuric acid. The emulsion was substantially freed of residual water soluble salts by washing by a conventional coagulation technique. After washing, 428 grams

of photographic gelatin and sufficient distilled water to bring the total weight to 7.8 kilograms were added and the emulsion was dispersed at 40° C. at a pH of 6.4. 114 cc. of a 10% solution of salicylamide were added and the emulsion was chemically sensitized as described in Example I. The mass was then cooled to 40° C. A coating aid was added and the emulsion was applied as a layer on cellulose acetate film support at the rate of 570 sq. ft. per mol of silver.

## EXAMPLE VI

An emulsion was prepared by the method described in Example II except that Solutions B and C were run into Solution A in approximately 2 minutes instead of 11 minutes. The silver halide grains obtained had an average size less than 1 micron diameter. An emulsion was obtained which, upon testing by the X-ray diffraction method of Berry, averaged less than 3.0 dislocations per micron<sup>2</sup> of silver halide surface area computed from the formula:

Concentration of dislocations

$$N = \frac{\Delta 2\theta}{bD \times 10^8} \text{ (per micron}^2\text{)}$$

in which

D is grain diameter in microns

b is the length of the Burger's vector

and

$\Delta 2\theta$  is the diffraction spot width in radians which is independent of the dimensions of the X-ray source.

Three strips of each of the photographic films as prepared in Examples I and II were given a positive exposure for  $\frac{1}{25}$  of a second in an Ib sensitometer and one sample of each after potassium ferricyanide bleach treatment was processed in an internal developer, a second of each in a surface developer, of the formulas given above, the development in the internal developer being for 5 minutes and that in the surface developer for 6 minutes. The third strips of each were given a cyan reversal development. The surface and internal sensitivities of the emulsion produced in accordance with the process of Example I were determined as described above. These sensitivities as expressed in log E values differed by somewhat less than 1.75. This difference as determined in the case of the emulsion produced in accordance with the process of Example II was well above 1.75 in terms of log E values.

The third strips of each of the films as prepared in Examples I and II after exposure was bathed in a prehardening bath for 3 minutes having the following composition:

|                           |       |     |
|---------------------------|-------|-----|
| Sodium hexametaphosphate  | grams | 0.5 |
| Sodium bisulfite          | do    | 10  |
| Formaldehyde 40% solution | cc    | 27  |
| Sodium carbonate          | grams | 10  |
| Sodium sulfate            | do    | 100 |
| Potassium bromide         | do    | 2.5 |
| Water to make 1 liter.    |       |     |

The strips were washed and then developed in a developer of the following composition for 8 minutes:

|                                |       |  |
|--------------------------------|-------|--|
|                                | Grams |  |
| Sodium hexametaphosphate       | 0.5   |  |
| Sodium sulfite                 | 40    |  |
| N-methyl-p-aminophenol sulfate | 5.0   |  |
| Hydroquinone                   | 2.0   |  |
| Sodium carbonate monohydrate   | 25    |  |
| Potassium bromide              | 1.1   |  |
| 1-phenyl-5-mercaptopotetrazole | 0.01  |  |
| Water to make 1 liter.         |       |  |

The film strips were washed and flashed to white light. The film strips were then developed in a cyan developer having the following composition:

|                                              |       |  |
|----------------------------------------------|-------|--|
|                                              | Grams |  |
| Sodium hexametaphosphate                     | 0.5   |  |
| Sodium sulfite (dessicated)                  | 5.0   |  |
| Isopropyl naphthalene sodium sulfonate       | 0.2   |  |
| 2-amino-5-diethylamino-toluene hydrochloride | 1.0   |  |

|                                                                    |      |
|--------------------------------------------------------------------|------|
| Sodium carbonate monohydrate                                       | 15.0 |
| Potassium bromide                                                  | 0.25 |
| Sodium hydroxide                                                   | 0.5  |
| 2,4 - dichloro - 5 - (p - toluene sulfonyl - amino - 1 - naphthol) | 1.4  |
| Sodium monohydroquinone sulfonate                                  | 0.6  |
| Water to make 1 liter.                                             |      |

The film strips were washed and then bleached in a bath having the following composition:

|                          |       |
|--------------------------|-------|
| 10                       | Grams |
| Sodium hexametaphosphate | 1     |
| Potassium ferricyanide   | 80    |
| Potassium bromide        | 40    |
| Water to make 1 liter.   |       |

The film strips were then thoroughly washed and dried. There was obtained a direct positive image in color. A determination of the maximum density showed the emulsion prepared in accordance with Example I to have a density of 3.10 and that from Example II greater than 4.6.

In the determination of the particle crystal dislocation by the formula

25 Number of particle crystal dislocations

$$N = \frac{(\Delta 2\theta)D}{b}$$

the diffraction spot value,  $\Delta 2\theta$ , in radians (also called angular misalignment) is determined conveniently by the X-ray diffraction method described in the Berry article in Journal of Applied Physics referred to above.

30 The particle diameter, D, is conveniently determined by observing the projected diameter in microns of the grains from a photomicrograph thereof and then dividing by the degree of magnification which was used. However, other methods of determining the particle diameters of the grains are available. For instance, this value may be determined by a method involving counting of 35 the number of spots as described in the book "X-rays in Practice" by Wayne T. Sproull, pages 440-446, McGraw-Hill, 1946.

40 The value b, length of the Burger's vector, is constant with the particular crystal type being considered. With the crystal structure of silver halide grains the 45 value b is 4.0 Angstrom units. Thus the formula for the determinations here is

$$N \text{ (per micron)} =$$

$$50 \frac{\text{width of diffraction spot (in radians)}}{4 \text{ times the particle diameter (in microns)} \times 10^8}$$

55 The invention has been described in considerable detail with particular reference to certain preferred embodiments thereof, but it will be understood that variations and modifications can be effected within the spirit and scope of the invention as described hereinabove, and as defined in the appended claims.

We claim:

60 1. A method of preparing photographic emulsions, the silver halide crystals of which have high surface and low internal sensitivity, which comprises mixing with an aqueous solution of a protein peptizer for silver halide, alkali metal halide in aqueous solution, which halide 65 essentially consists of bromide and iodide of which the latter constitutes 0.5-5 mole percent and ammoniacal silver nitrate, at least 50% of the alkali metal halide which reacts with the ammoniacal silver nitrate being added simultaneously therewith to the protein peptizer 70 solution over a period of not more than 20 minutes, removing residual water soluble salts from the silver halide crystals which are formed thereby and digesting the mass to a selected photosensitivity.

75 2. A method of preparing photographic emulsions, the silver halide crystals of which have high surface and

low internal sensitivity, which comprises mixing with an aqueous solution of a protein peptizer for silver halide, alkali metal halide in aqueous solution, which halide essentially consists of bromide and iodide of which the latter constitutes 0.5-5 mole percent, and ammoniacal silver nitrate, at least 50% of the alkali metal halide which will react with the silver nitrate being added simultaneously therewith to the protein peptizer solution over a period of not more than 20 minutes, removing residual water soluble salts from the silver halide crystals formed thereby and digesting those crystals with a sulfur sensitizer to a selected photosensitivity.

3. A method of preparing photographic emulsions, the silver halide crystals of which have high surface and low internal sensitivity, which comprises mixing with an aqueous solution of a protein peptizer for silver halide, alkali metal halide in aqueous solution, which halide essentially consists of bromide and iodide of which the latter constitutes 0.5-5 mole percent, and ammoniacal silver nitrate, at least 50% of the alkali metal halide which reacts with the ammoniacal silver nitrate being added simultaneously therewith to the protein peptizer solution over a period of not more than 20 minutes, removing residual water soluble salts from the silver halide crystals formed thereby and digesting those crystals with a sulfur sensitizer and a gold sensitizer to a selected photosensitivity.

4. A method of preparing photographic emulsions, the silver halide crystals of which have high surface and low internal sensitivity, which comprises mixing with an aqueous solution of gelatin, alkali metal halide in aqueous solution, which halide consists of bromide and iodide of which the latter constitutes 0.5-5 mole percent, and ammoniacal silver nitrate, at least 50% of the alkali metal halide which reacts with the ammoniacal silver nitrate being added simultaneously therewith to the aqueous gelatin solution over a period of not more than 20 minutes, removing residual water soluble salts from the silver halide crystals formed and digesting the silver halide crystals with a sulfur sensitizer and a gold sensitizer to a selected photosensitivity.

15

5

10

20

25

#### References Cited by the Examiner

##### UNITED STATES PATENTS

|           |         |              |       |       |
|-----------|---------|--------------|-------|-------|
| 2,456,956 | 12/1948 | Knott et al. | ----- | 96-22 |
| 2,490,751 | 12/1949 | Hanson       | ----- | 96-19 |

##### OTHER REFERENCES

Hedges et al., Philosophical Magazine, vol. 44, Series 7, 1953, p. 369.

NORMAN G. TORCHIN, Primary Examiner.

J. RAUBITSCHEK, Assistant Examiner.

UNITED STATES PATENT OFFICE  
CERTIFICATE OF CORRECTION

Patent No. 3,276,877

October 4, 1966

Henry Clay Yutzy et al.

It is hereby certified that error appears in the above numbered patent requiring correction and that the said Letters Patent should read as corrected below.

Column 3, line 41, for "2,423,459" read -- 2,423,549 --; column 6, lines 57 and 68, column 7, lines 9, 18, 33, 38, 42, 47, 50 and 58, insert as a heading over the right-hand column, each occurrence, -- 1 Liter --; column 7, line 1, before ".02" insert -- gm --; column 8, line 49, for "dissolved" read -- dissolved --.

Signed and sealed this 5th day of September 1967.

(SEAL)

Attest:

ERNEST W. SWIDER  
Attesting Officer

EDWARD J. BRENNER  
Commissioner of Patents